

## [54] BISMUTH-TIN-INDIUM ALLOY

[75] Inventors: Hideki Murabayashi, Kawasaki; Katsuhiko Kawakita, Yokosuka; Kisaku Nakamura, Funabashi; Sadao Kobatake, Yokohama, all of Japan

[73] Assignee: Tokyo Shibaura Electric Co., Ltd., Japan

[\*] Notice: The portion of the term of this patent subsequent to Apr. 11, 1995, has been disclaimed.

[21] Appl. No.: 851,267

[22] Filed: Nov. 14, 1977

## Related U.S. Application Data

[63] Continuation of Ser. No. 668,448, Mar. 19, 1976, abandoned.

## [30] Foreign Application Priority Data

Mar. 20, 1975 [JP] Japan ..... 50-32937

[51] Int. Cl.<sup>2</sup> ..... C22C 12/00  
[52] U.S. Cl. ..... 75/134 D; 75/134 B;  
176/86 M

[58] Field of Search ..... 75/134 K, 134 B, 134 D,  
75/134 N, 134 R, 134 T, 166 B, 166 C, 175 R,  
175 A; 176/37, 87, 88

## [56]

## References Cited

## U.S. PATENT DOCUMENTS

|           |        |                          |          |
|-----------|--------|--------------------------|----------|
| 2,117,282 | 5/1938 | Austin .....             | 75/175 A |
| 2,636,820 | 4/1953 | Bolton .....             | 75/175 R |
| 2,649,367 | 8/1953 | Smith et al. .....       | 75/134 T |
| 2,649,368 | 8/1953 | Smith et al. .....       | 75/134 T |
| 2,649,369 | 8/1953 | Smith et al. .....       | 75/134 T |
| 3,269,735 | 8/1966 | Whittaker .....          | 176/79   |
| 4,083,718 | 4/1978 | Murabayashi et al. ..... | 75/134 D |

## FOREIGN PATENT DOCUMENTS

48-39694 11/1973 Japan

## OTHER PUBLICATIONS

Cooper, L. P. et al.; *Operating Experience with the EBR-II Rotating-Plug Freeze Seals*; Argonne National Laboratory ANL-7617, pp. 19-20 (12/69).

Primary Examiner—L. Dewayne Rutledge

Assistant Examiner—Michael L. Lewis  
Attorney, Agent, or Firm—Finnegan, Henderson, Farabow, Garrett & Dunner

## [57]

## ABSTRACT

Disclosed is a bismuth-tin-indium alloy consisting essentially of 53 to 76 weight % of bismuth, 22 to 35 weight % of tin and 2 to 12 weight % of indium. This alloy has excellent sealing property and oxidation resistance, and is suitable particularly to the use as a seal material for a rotating plug of a nuclear reactor.

2 Claims, 3 Drawing Figures



FIG. 1



FIG. 2





## BISMUTH-TIN-INDIUM ALLOY

This is a continuation of application Ser. No. 668,448, filed Mar. 19, 1976, now abandoned.

## BACKGROUND OF THE INVENTION

This invention relates to an alloy having a low melting point usable as a seal material for a metal-made vessel such as a vessel formed of stainless steel, and more particularly to a Bi-Sn-In alloy.

Conventionally, an alloy having a low melting point is employed as a seal material for use in a metal-made vessel such as a vessel formed of stainless steel. For example, a rotating plug 2 of a reactor vessel 1 shown in FIG. 1 is required to be sealed for purpose of preventing the leak-out into the atmosphere of a cover gas 4 having radio activity covering the upper surface of a coolant 3 within the reactor vessel 1. The sealing of the rotating plug 2 is effected by providing a circular blade 5 attached to an edge portion of the plug 2, respectively and immersing this blade within a trough 6 in which is received a fusible seal material 7 consisting of a low-melting alloy.

A Bi-Sn eutectic composition (Bi 57 weight %, Sn 43 weight %) is conventionally known as a seal material. This alloy has as high a melting point as about 140° C., and simultaneously has no good sealing property. Further, a fusible seal material is also known whose melting point, i.e., solidification starting point is reduced to 100° C. or less by adding a large amount of In to the Bi-Sn eutectic composition alloy. This alloy has Bi-Sn-In proportion of 60 to 64 weight %, 17 to 21 weight % and 17 to 21 weight %, respectively, and a solidification starting point of 79 to 89° C., and has degraded sealing property and low oxidation resistance, and in addition uneconomically requires a large amount of In. Assume now that a Bi-Sn-In alloy having said proportion be used as a seal material for sealing the rotating plug 2 of the reactor vessel 1 shown in FIG. 1. Upon performing the rotation operation of the rotating plug 2, the seal material 7 is molten while during a normal operation of the reactor vessel the seal material 7 is solidified to fixedly hold the plug 2 in place. Since, in this case, the seal material 7 exhibits no sufficient degree of sealing property when having been solidified, a complete sealing of the plug 2 during the reactor vessel operation can not be expected. Further, during a period in which the seal material 7 is molten, that is, during the plug rotation, the seal material 7 is oxidized, for which reason the composition of the seal material is varied to decrease the reliability upon a condition in which the cover gas 4 within the reactor vessel 1 is sealed. Under such circumstances, there has been a demand for an inexpensive seal material having excellent sealing property and oxidation resistance.

## SUMMARY OF THE INVENTION

An object of the invention is to provide a Bi-Sn-In alloy which is low in manufacturing cost and excellent in terms of sealing property and oxidation resistance.

Another object of the invention is to provide a Bi-Sn-In alloy having a solidification starting point of about 100° to 150° C.

Still another object of the invention is to provide a Bi-Sn-In alloy for use as a fusible seal material for sealing a rotating plug of a reactor vessel.

Other objects and advantages will become apparent from the following detailed description and claims.

According to the invention, there is provided a Bi-Sn-In alloy consisting essentially of 53 to 76 weight % of Bi, 22 to 35 weight of Sn and 2 to 12 weight % of In, or more preferably a Bi-Sn-In alloy consisting essentially of 56 to 73 weight % of Bi, 25 to 32 weight % of Sn and 2 to 12 weight % of In.

## BRIEF DESCRIPTION OF THE DRAWING

FIG. 1 is a sectional view of a reactor vessel, showing the condition wherein an alloy according to the invention is applied as a sealing material for a rotating plug of the reactor vessel;

15 FIG. 2 is a triangular diagram showing the sealing property as measured by color-check method, of a Bi-Sn-In alloy having various proportions; and

20 FIG. 3 is a graph showing the result of a gas-leak test in correlation to the measured result obtained by color-check method.

## DETAILED DESCRIPTION OF THE INVENTION

Preferred embodiments of the invention are hereinafter explained while they are being compared with controls.

25 Samples of a Bi-Sn-In alloy having a wide variety of proportions were prepared, and the sealing property and oxidation resistance of the individual samples were 30 determined in accordance with the following tests.

## TEST OF SEALING PROPERTY

This test was carried out in accordance with the following two methods. Generally, the sealing property 35 of a metal seal has a tendency to become lower under a solid condition than under a liquid condition. Therefore, the test was performed under a solid condition with respect to all samples. The test was conducted under the condition of the sample thickness being 10 40 mm.

## 1. Color Check Method

First, in order to model an actual sealing mechanism a sample was poured for casting into a stainless steel-made crucible at a central part of which a stainless steel plate was installed. Subsequently, after heated at 150° C. for 75 hours, the sample was allowed to cool and an inner bottom surface of the crucible was abraded for removal of the bottom. Next, through allowing red ink to flow on the sample surface from the opening of the crucible and allowing the resulting sample to stand in the atmosphere for 16 hours and then applying a white developing solution on the exposed bottom surface of the sample, the sealing property of the sample was investigated while observing the existence or non-existence of the red ink at the contact portions between the sample and the crucible and between the sample and the stainless steel plate. Although the test of sealing property by color check is qualitative, the precision with which the sealing property was judged was higher than that attainable with a gas-leak method as later described.

## 2. Gas-leak Method

This method is for purpose of quantitatively measuring the sealing property. In replacement of the stainless steel plate used in the color check method, a stainless steel tube was installed within a crucible. That is, one end of the stainless steel tube is kept closed by a Bi-Sn-In alloy. First, the tube interior was vacuumized

from the other end of the tube and was filled with an argon gas, and thereafter was increased up to a pressure of 1 kg/cm<sup>2</sup> (gauge pressure). Then, the resulting tube was allowed to stand and the value of pressure reduction with time was recorded.

As stated in the above item 1, the precision of judging the sealing property is higher than that attainable with the gas-leak method. The sealing property of the sample was measured by colorcheck method, the result being classified into four types- "very good", "good", "rather bad" and "bad" and presented in Table as later shown. The relationship between this measured result and the result quantitatively obtained with gas-leak method is indicated in FIG. 3.

Next, the method of testing the oxidation resistance of the sample is explained.

#### Oxidation test

20 Grams of each sample of Bi-Sn-In alloy having various proportions of Bi, Sn and In were poured for casting into a magnetized crucible and held in the atmosphere at a temperature of 150° C. for 280 hours. And the surface condition of each sample was observed. The measured result of oxidation resistance of the sample was classified into four types- a "very good" sample presenting no color variation, a "good" sample presenting little color variation, a "rather bad" sample which is a light blackened one, and a "bad" sample which is a deep blackened one.

The respective results of the above-mentioned sealing property test and oxidation test are shown in Table 30 below. In Table, sample Nos. 2 to 13 are Bi-Sn-In alloys according to the invention while sample Nos. 1 and 14 to 16 Bi-Sn-In alloys according to controls.

Table

| Sample No. | Proportion weight % |    |    | Oxidation resistance | Sealing property |
|------------|---------------------|----|----|----------------------|------------------|
|            | Bi                  | Sn | In |                      |                  |
| 1          | 74                  | 25 | 1  | Very good            | Rather bad       |
| 2          | 76                  | 22 | 2  | Good                 | Good             |
| 3          | 67                  | 30 | 3  | Very good            | Very good        |
| 4          | 65                  | 30 | 5  | Very good            | Very good        |
| 5          | 60                  | 35 | 5  | Very good            | Good             |
| 6          | 68                  | 22 | 10 | Very good            | Good             |
| 7          | 65                  | 25 | 10 | Very good            | Good             |
| 8          | 60                  | 30 | 10 | Very good            | Very good        |
| 9          | 58                  | 32 | 10 | Very good            | Very good        |
| 10         | 63                  | 25 | 12 | Very good            | Very good        |
| 11         | 61                  | 27 | 12 | Very good            | Very good        |
| 12         | 58                  | 30 | 12 | Very good            | Very good        |
| 13         | 53                  | 35 | 12 | Very good            | Good             |
| 14         | 65                  | 20 | 15 | Bad                  | Rather bad       |
| 15         | 62                  | 21 | 17 | Bad                  | Bad              |
| 16         | 50                  | 25 | 25 | Bad                  | Bad              |

Solidification starting point is set at 109.5° C. when the sample has a Bi-Sn-In proportion of, for example, 60 weight %, 30 weight % and 10 weight %, respectively.

As apparent from the above Table, a Bi-Sn-In alloy having a proportion of 53 to 76 weight %, 22 to 35 weight % and 2 to 12 weight %, respectively, is excellent in terms of both oxidation resistance and sealing property. It should be noted that the alloys set out in the above Table are substantially lead-free. This Bi-Sn-In alloy is extremely excellent, more preferably at 56 to 73 weight %, 25 to 32 weight % and 2 to 12 weight %, respectively. When this proportion range is shown by means of a triangular diagram, it is indicated by a region surrounded by a solid line 8 of FIG. 2. The measured result of the sealing property as classified into the above-mentioned four types or stages is indicated at positions corresponding to the respective proportions within the triangular diagram in such a manner that a

proportion corresponding to said "very good" sample is indicated by a mark "o", a proportion corresponding to said "good" sample by a mark  $\Delta$ , a proportion corresponding to said "rather bad" sample by a mark  $\blacktriangle$  and a proportion corresponding to said "bad" sample by a mark x.

As seen from Table, any Bi-Sn-In alloy having an In content of 12 weight % or less exhibits excellent oxidation resistance. The In content of 12 weight % is indicated by a dotted line within the triangular diagram of FIG. 2. If, however, the In content is less than 2 weight %, the resulting sample has degraded sealing property and is unsuitable to the practical use.

As already stated, the measurement of the sealing property was made by color-check method, and the relationship between this measured result and the result of the gas-leak test is shown in the graph of FIG. 3. In this graphic diagram, the marks o,  $\Delta$ ,  $\blacktriangle$  and x correspond to the measured result obtained by color-check method, i.e., "very good", "good", "rather bad" and "bad", respectively.

The Bi-Sn-In alloy according to the invention exhibits its effectiveness particularly when used as a seal material for sealing a rotating plug of the reactor vessel. That is, since the solidification starting point of the Bi-Sn-In alloy ranges from 100° C. to 150° C., the sealing property thereof is not weakened by a temperature rise during the operation of the reactor vessel. Further, the stainless steel constituting the material of the reactor vessel, when temperature exceeds 150° C., increases in thermal stress to decrease in intensity. However, if the alloy according to the invention is used as a seal material for the rotating plug, since its melting point is low, there is no necessity of heating the seal material up to such a high temperature during the rotation of the rotating plug. Accordingly, too high a stress is not applied to the stainless steel of the reactor vessel.

Note that even though incidental impurities are contained in the Bi-Sn-In alloy according to the invention, it will not depart from the scope of the invention.

Since, as above described, the Bi-Sn-In alloy according to the invention has extremely excellent sealing property and oxidation resistance and is not required to contain a large amount of expensive indium, it is very economical. For this reason, the alloy according to the invention is very suitable to the use as a seal material for sealing the rotating plug of the reactor vessel. Further, the alloy according to the invention is usable not only as a seal material for sealing a stainless steel-made vessel but also as a seal material for bonding or sealing a metallic member formed of aluminium-based alloy, copper-based alloy, etc. Furthermore, since the alloy according to the invention has low melting point and is excellent in terms of property permitting the adhesion between metallic members, it can suitably be employed as a safety valve of vessel such as a pressurized cooker.

What we claim is:

1. A substantially lead free low melting point, sealing alloy of bismuth, tin and indium which consists essentially of 53 to 76 weight percent bismuth, 22 to 35 weight percent tin and 2 to 12 weight percent indium, said alloy being substantially resistant to atmospheric oxidation at temperatures up to 150° C.

2. A substantially lead free low melting point, sealing alloy of bismuth, tin and indium which consists essentially of 56 to 73 weight percent bismuth, 25 to 32 weight percent tin and 2 to 12 weight percent indium, said alloy being substantially resistant to oxidation at temperatures up to 150° C.

\* \* \* \* \*